# EUROPEAN PATENT SPECIFICATION

(11) **EP 2 683 839 B1**
(45) Date of publication and mention of the grant of the patent: **01.04.2015**
(21) Application number: 12708008.3
(22) Date of filing: 07.03.2012
(51) Int. Cl.: C21D 8/02, C21D 9/46, C22C 38/04, C23C 2/06, C23C 2/28, C23C 2/02

(54) **PROCESS FOR PRODUCING HIGH STRENGTH FORMABLE STEEL AND HIGH STRENGTH FORMABLE STEEL PRODUCED THEREWITH**
VERFAHREN ZUR HERSTELLUNG VON HOCHFESTEM FORMBAREM STAHL UND DAMIT HERGESTELLTER HOCHFESTER FORMBARER STAHL
PROCÉDÉ POUR PRODUIRE UN ACIER FORMABLE À HAUTE RÉSISTANCE ET ACIER FORMABLE À HAUTE RÉSISTANCE PRODUIT PAR CELUI-CI

(30) Priority: 07.03.2011 EP 11157239
(43) Date of publication of application: 15.01.2014
(73) Proprietor: Tata Steel Nederland Technology B.V., NL-1951 JZ VELSEN-NOORD (NL)
(72) Inventor: HANLON, David Neal, NL-1970 CA Ijmuiden (NL); VAN BOHEMEN, Stefanus Matheus Cornelis, NL-1970 CA Ijmuiden (NL)
(74) Representative: Bodin, Andre
(86) International application number: PCT/EP2012/053856
(87) International publication number: WO 2012/120020

(56) References cited:
- EP-A1- 1 707 645
- EP-A1- 1 724 371
- EP-A1- 2 202 327
- WO-A1-2010/029983
- JP-A- 2003 013 177
- COOMAN DE B C ET AL: "MECHANICAL PROPERTIES OF LOW ALLOY INTERCRITICALLY ANNEALED COLD ROLLED TRIP SHEET STEEL CONTAINING RETAINED AUSTENITE", CANADIAN METALLURGICAL QUARTERLY, TARRYTOWN, NY, US, vol. 43, no. 1, 1 January 2004 (2004-01-01), pages 13-24, XP009031577,

## Description

### FIELD OF THE INVENTION

The invention relates to a method for producing a steel strip composite and to a steel strip composite produced by said method.

### BACKGROUND OF THE INVENTION

Enhancement of ductility at elevated strength is desirable for widespread markets.

In the automotive industry in particular, where legislation is driving improvements in fuel economy and safety, there is a move towards stronger, formable high strength steels. High strength and ultrahigh strength strip steel provides automotive manufacturers potential for down weighting of the body in white and the opportunity for countering weight increases arising from the move to electric and hybrid vehicles. In addition high and ultrahigh strength steels play a critical role in determining the crash worthiness of modern passenger vehicles.

Extensive application of high strength and ultrahigh strength steel requires, in many cases, levels of formability that are higher than can be expected for conventional carbon-manganese steels. Enhancement of residual ductility in formed parts is beneficial for integrity in crash. As a first approximation tensile elongation may be considered a simple measure of both formability and impact integrity. Consequently, such effort has been given to developing advanced high strength steels (AHSS) with optimised tensile ductility.

In the case of current commercial AHSS, enhancement of ductility is realised either by using composite effects (Dual Phase or DP steels) or by using deformation induced transformation of retained austenite (TRIP steels). Both composite hardening and transformation induced plasticity mechanisms can measurably enhance the ductility of predominantly ferritic steels. However, the enhancement of ductility which may be achieved in this way is limited to around 1.5 (for DP) to 2 (for TRIP) times that of conventional C-Mn steels at equivalent strength. Furthermore, the strength level that may be achieved in commercial, ferritic-matrix DP and TRIP steels is also limited (TRIP to around 800MPa and DP to around 1000MPa).

Extreme enhancement of tensile ductility may also be achieved by utilising high alloy (predominantly manganese) additions to stabilise austenite (Twinning Induced Plasticity or TWIP steels). Austenite is inherently more ductile than ferrite and twinning provides a very effective work hardening mechanism. Such steels may achieve very high elongations (typically 50%) at very high strengths (typically 1000MPa). The improvement in elongation may be typically 5x that of a conventional C-Mn steel. However, the yield strength is comparatively low and large strains need to be uniformly imposed to achieve high strength in the formed component. Furthermore, the extremely high levels of alloy make large scale production over conventional process problematic.

Practical experience gained during the implementation of these first and second generations of AHSS have revealed that forming and performance parameters beyond those measured in the tensile test can represent significant barriers to implementation. In particular, although exhibiting high uniform and total elongations, and consequently high resistance to necking during stretch forming, mixed microstructures comprising a distribution of hard phase in a matrix of soft ferrite may be highly susceptible to cracking at stretched edges. Low stretched edge formability is known to impose a practical limit to the formability of otherwise highly ductile AHSS.

WO2010/029983 discloses a method for manufacturing a high-strength steel sheet, comprising hot-rolling and then cold-rolling a billet to be formed into a steel sheet having the composition on a mass percent basis: 0.17%-0.73% C; 3.0% or less Si; 0.5%-3.0% Mn; 0.1% or less P; 0.07% or less S; 3.0% or less Al; 0.010% or less N, balance Fe and incidental impurities to form a cold-rolled steel sheet, annealing the cold-rolled steel sheet in an austenite single-phase region for 15 seconds to 600 seconds, cooling the cold-rolled steel sheet to a first temperature range of 50 °C to 300 °C at an average cooling rate of 8 °C/s or more, heating the cold-rolled steel sheet to a second temperature range of 350 °C to 490 °C, and maintaining the cold-rolled steel sheet at the second temperature range for 5 seconds to 1000 seconds.

A new generation of AHSS that exhibits an advantage in strength ductility-balance with respect to carbon manganese steels but at lower levels of alloy, and consequently lower cost and greater processability, is emerging. For this generation of steels more attention is also being paid to other formability parameters such as stretched edge ductility (hole expansitivity) and bendability. In most cases, mixed microstructures comprising hard majority phases such as martensite or bainite are used to develop high to ultrahigh strengths. Such hard, uniformly fine, microstructures tend to exhibit good hole expansitivity. Alloy compositions fall into two basic categories: Medium Manganese compositions (Mn typically 7wt%) and Medium Carbon, carbon-manganese steels with additions of Si and or Al.

In the case of the high Mn TRIP steels austenite is simply chemically stabilised by large additions of Mn. Although clearly differentiated strength-ductility combinations can be achieved in this way, processing has proven to be difficult since hard, brittle martensitic phases are developed in intermediate product. This renders further processing, such as cold rolling, difficult at dimensions relevant to commercial processing. Furthermore, alloy costs are high due to the high manganese content.

Therefore the problem arises that it is difficult to provide a steel strip having improved strength and edge ductility.

It is an object of this invention to provide a method for improving the strength and edge ductility of steels.

It is a further object of this invention to provide a steel having improved strength and ductility in combination with an low allow content.

### SUMMARY OF THE INVENTION

According to a first aspect of the invention there is provided a method for producing a quenched and partitioned steel by providing a cold rolled and annealed steel strip containing (in weight %):
- 0.18 - 0.4% C
- 1.5 - 4.0% Mn
- 0.5 - 2.0% Si
- 0 - 1.5% Al
- 0 - 0.5% Mo
- 0 - 0.5% tri
- 0 - 0.4% V
- 0 - 0.010% Nb
- 0 - 0.005% B
- 0 - 0.015% N
- 0 - 0.08% P
- 0 - 0.01% S
- 0 - 0.06% Sb
- 0 - 0.05% Ca.
- 0 - 1.0%Cr
- 0 - 1.0% Ni
- the remainder being iron and unavoidable impurities.
wherein the annealing process comprises the following steps:
(i) reheating the cold rolled strip to an annealing temperature T₁ of between Ac₃-40 and Ac₃+80;
(ii) holding the strip at T₁ for an annealing time t₁ of between 10 and 200 seconds;
(iii) cooling the annealed strip at a cooling rate CR1 to a quench temperature T₂ for producing a microstructure in the strip comprising a martensite fraction and a retained austenite fraction;
(iv) partitioning annealing the cooled strip at a temperature T₃ for enriching the austenite in carbon by repartitioning the carbon from the martensite to the austenite fraction for a repartitioning time t₂ of between 20 and 500 seconds;
(v) cooling the strip at a cooling rate CR2 to ambient temperature.

According to the invention a cold-rolled strip is provided by the conventional and known processes of casting, hot-rolling and cold-rolling. The casting process may involve thick slab casting (slab thickness between 150 and 350 mm), thin slab-casting (slab thickness below 150 mm, usually between 50 and 100 mm) or even strip casting. Cold rolling is also a conventional and known process.

The composition of the steel according to the invention is a balanced composition comprising medium carbon and moderate manganese additions. The cold rolled steel is heated to form austenite, either partially or fully, followed by quenching to a temperature between the martensite start temperature (Mₛ) and the martensite finish temperature (M_{f}), thereby creating a controlled amount of martensite and retained austenite. The manganese additions result in stabilisation of an austenite fraction during cooling from the annealing temperature and the subsequent carbon enrichment further stabilises the austenite fraction. Combined stabilisation via C and Mn additions enables alloying with either element to be restricted to reasonable limits leading to cost and processability advantages. The steel is then subjected to a thermal treatment to partition carbon from the martensite into the austenite. The carbon enrichment of the austenite fraction is achieved by partitioning from martensite or low temperature bainitic transformation or preferably a combination of both. By this partitioning, the formation of carbides is suppressed and the austenite is stabilised rather than decomposed. Combined stabilisation with partitioning and bainitic transformation enables the amount of austenite and the microstructure in which it is embedded to be optimised. The bainitic transformation also leads to carbon enrichment of the remaining austenite because the formation of carbides is suppressed. All compositions are given in weight percentages, unless otherwise indicated. The final microstructure of the steel comprises martensite, bainite and carbon-enriched austenite and, if T₁ < Ac₃, equiaxed ferrite. The stabilisation of austenite results in the steel exhibiting improved ductility relative to traditional high strength steels.

Carbon (C) provides solid solution strengthening, enhances hardenability (thus enabling avoidance of high temperature transformations at cooling rates achievable in conventional annealing lines) and, when dissolved in austenite, promotes the retention of austenite at room temperature. Above 0.4wt% C the propensity for formation of brittle high carbon martensite increases.

Manganese (Mn) delivers substantial solid solution strengthening, stabilises austenite, thus promoting its retention at room temperature, and enhances hardenability promoting the formation of hard transformation products at cooling rates achievable in conventional annealing lines. A preferable upper limit for the manganese content is 3.5%.

Silicon (Si) addition provides solid solution strengthening thus enabling the attainment of high strength and promotes the stabilisation of austenite. Si very effectively retards the formation of carbides during overaging thus keeping carbon in solution for stabilisation of austenite. Ferrite and hard phases such as bainite and martensite exhibit improved ductility in the absence of carbides. Free carbon, not trapped in carbides, may be partitioned to austenite. For acceptable coatability the imposed addition of Si should be below a certain level: Si may be added in the range of between 0.5 to 1wt% when combined with Al addition. In the absence of Al additions beyond the level needed for deoxidation Si should be maintained in the range of between 1 to 2wt%.

Aluminium (Al) is usually already added in small quantities of at most 0.1% and preferably at most 0.05% to liquid steel for the purpose of deoxidation by forming alumina. Ideally, the total aluminium content in the steel is between 0.01 and 0.08% if aluminium is only added for desoxidation. In the right quantity it also provides an acceleration of the bainite transformation. Al also retards the formation of carbides thus keeping carbon in solution for partitioning to austenite and promoting the stabilisation of austenite. A maximum value of 1.5wt% is imposed for castability purposes because higher Al-contents lead to poisoning of casting mould slag and consequently an increase in mould slag viscosity leading to incorrect heat transfer and lubrication during casting. Aluminium alone delivers low strength. Therefore, if Al is used above levels required for deoxidation it should always be in combination with Si.

Niobium (Nb), if added, is added in small amounts of up to 0.1% or more preferably of up to 0.05wt%. It is added for austenitic grain refinement during hot rolling. If combined with a suitable rolling schedule, it promotes transformation on the run-out-table, and thus finer and a more homogeneous grain size in the hot-rolled intermediate product which is then subsequently cold-rolled.

Titanium (Ti) can be used to form fine precipitates in the ferritic component of mixed microstructures thus increasing strength and promoting uniformity of strength at the microstructural scale and in turn good stretched edge ductility. Preferably Ti is below 0.1%.

Molybdenum (Mo) is used to increase hardenability thus retarding the formation of high temperature transformation products on cooling to the quench temperature. Additions of Mo may therefore allow the utilisation of lower cooling rates more readily achieved in full-scale production lines or to achieve the desired structure and properties in heavier gauge strip. The use of Mo is to be preferred over the use of Cr when UHS is required since in addition to enhancing hardenability Mo provides additional solid solution strengthening. Mo is also known to retard coarsening of fine strengthening precipitates thus promoting thermal stability precipitation strengthening variants. For reasons of cost less than 0.5wt% is preferable.

Vanadium (V) is used to increase hardenability thus retarding the formation of high temperature transformation products on cooling to the quench temperature. Furthermore V may combine with C or N or both to form fine strengthening precipitates thus increasing strength and promoting uniformity in strength at the microstructural scale in mixed microstructures and in turn improved stretched edge ductility. V addition up to 0.4wt% is effective. Higher additions are undesirable for reasons of cost and because excessive levels of precipitation tie up high amounts of C. Since free C is required for austenite stabilisation too high V requires increased C addition. Preferably V is below 0.1%.

Phosphorus (P) is used to suppress the formation of pearlite during cooling, to suppress carbide formation and thereby promote the partitioning of carbon to austenite resulting in austenite stabilisation. However, too high a P addition is known to cause embrittlement at hot-rolling temperatures and to lead to reduced toughness in martensitic UHSS. P may also lead to problems in spot welding of the final product. For these reasons P is limited to a maximum of 0.08wt% and more preferably to a maximum of 0.02wt%.

Sulphur (S) is an impurity which may embrittle the intermediate or final product. S should be limited to a maximum level of 0.01wt% and more preferably to at most 0.005wt%.

Chromium (Cr) and nickel (Ni) may be used to increase hardenability thus retarding the formation of high temperature transformation products on cooling to the quench temperature. Additions of Cr and/or Ni may therefore allow the utilisation of lower cooling rates more readily achieved in full-scale production lines or to achieve the desired structure and properties in heavier gauge strip. Cr and/or Ni should be limited to a level of less than 1wt% for reasons of cost and preferably to levels of 0.5wt% or less and more preferably below 0.1%.

Boron (B) may be used to improve hardenability and, in particular, to prevent the formation of ferrite on cooling from a fully austenitic soaking temperature. B should be limited to 50ppm because above these levels further addition is ineffective.

Antimony (Sb) may be used to enhance the wettability of zinc during hot dip galvanising. Addition should be limited to 0.06wt% or less.

Calcium (Ca) may be required to avoid clogging during casting and may be beneficial for modifying the morphology of MnS inclusion. Globular inclusions are known to be less detrimental to stretched edge ductility than highly elongated inclusions If used, then addition should preferably be made to the level of 30ppm or less. Additions above 0.05% lead to the formation of coarse inclusions detrimental to ductility and toughness.

Nitrogen (N) may be used, in combination with V, to form fine strengthening precipitates imparting strength and promoting uniformity in strength at the microstructural scale and in turn good stretched edge ductility. Additions should be limited to 150ppm or less.

The annealing step starts with reheating to an annealing temperature (T₁). T₁ may be above or below Ac₃. If T₁ is below Ac₃ the resulting ferrite fraction leads to a lower strength and may introduce heterogeneity in strength at a microstructural scale. Local differences in strength lower the ratio of yield to tensile strength and lead to poor stretched edge ductility and bendability. It is therefore preferable that T₁ is above Ac₃. In the context of this invention the phrase "above Ac₃" means that the microstructure is austenitic at T₁. Although the equilibrium transformation temperature Ae₃ is only determined by the composition, the value of the corresponding Ac₃ temperature is not a constant value as its value depends among others on the heating rate during which Ac₃ is measured and the starting microstructure of the steel. Usually Ac₃ is determined using dilatometry. When the heating rate used during dilatometry and the microstructure of the test specimen are those used in the process according to the invention, the value of Ac₃ is easy to determine. In determining T₁ and the allowable variation around T₁ the narrowing of the transformation temperature range with increasing C content should preferably be taken into account as follows: $\left({AC}_{3}-40\right) < {T}_{1} \leq \left({AC}_{3}+50\right) for carbon between 0.18 - 0.3 % C$ or $\left({AC}_{3}-20\right) < {T}_{1} \leq \left({AC}_{3}+30\right) for carbon between 0.3 to 0.4 % C$

The rapid cooling to T₂ (CR1) is required to avoid the formation of high temperature transformation phases. The specific rate required depends upon the steel chemistry and corresponds to the critical cooling rate for avoidance of ferrite and pearlite noses in the relevant CCT diagram. In addition, the critical rate decreases with increasing T₁ above Ac₃. Preferably CR1, i.e. the cooling rate over the temperature interval 800-500°C from T₁ to T₂ is between 30 to 80 °C/s. T₂ should be chosen low enough to deliver partial transformation to martensite, but not so low as to cause complete transformation to martensite. T₂ is chosen to deliver a volume fraction of martensite of between 50 to 90% (in volume) and preferably an austenite fraction of at least vol.5%. The dependency of the martensitic transformation start temperature (M_{S}) on composition means that T₂ will also depend upon chemistry. Preferably a martensite fraction of 60 - 85 vol.% is chosen.

Holding at T₃ is needed to enrich the remaining austenite in carbon via a bainitic transformation or carbon partitioning or both. This temperature may be the same as the quench stop temperature (T₂=T₃) or may be higher (T₃>T₂). Higher isothermal holding temperatures may be advantageous since increased rates of carbon diffusion may make feasible shorter isothermal holds. Several processes occur during isothermal holding including tempering of martensite, diffusion of carbon from the martensite fraction to the remaining austenite, the precipitation of carbides and the formation of bainite. The presence of a small fraction of martensite is known to accelerate subsequent transformation to bainite so, for some combinations of alloy composition and processing capability, quench stop temperatures under Ms are desirable. T₃ is chosen so as to give a suitable rate of transformation to bainite or rate of partitioning or both. The specific temperature will be dependent upon alloy composition and will preferably fall in a range expressed by: $\left(Ms-70\right) < {T}_{3} \leq \left(Ms+150\right) , { and preferably T}_{3} \leq \left(Ms+50\right)$

The correct balance of isothermal holding temperature and isothermal holding time must be chosen for each composition. These can be determined by means of dilatometry as described hereinbelow.

The formation of carbides may lock up carbon which would otherwise be available for stabilisation of austenite and should therefore preferably be avoided. Furthermore, coarse Fe₃C carbides may lead to a deterioration in tensile ductility and/or stretched edge ductility. The levels of Si or Si/Al must be suitably tuned to retard carbide formation for the duration of the isothermal hold.

Since both the carbon partitioning accompanying the martensite tempering and bainitic transformation, in the presence of sufficient Si or Si/Al, each deliver an enrichment of carbon in austenite, exploitation of both mechanisms in tandem is highly beneficial leading to a greater total degree of austenite stabilisation.

It should also be noted that the optimum properties are not delivered by simply tuning process to deliver the maximum stabilisation of austenite. Levels of carbon enrichment too low to completely stabilise all austenite but sufficient to deliver high carbon austenite prior to the final cool can lead to the formation of brittle martensite. Excessive tempering of martensite can lead to significant loss in strength and, in combination with insufficient stabilisation of austenite and the formation of new hard martensite on final cooling, to low ratios of the yield to tensile strength.

Therefore, it is preferred that the partitioning temperature and time are chosen such as to optimise the enrichment of carbon in the austenite but without creation of deleterious microstructures during the isothermal hold.

Subsequent to the hold at T₃ the strip is cooled to ambient temperature. The strip may also be coated with zinc or other such metallic layers using a suitable method of deposition either in-line or in a following process step.

In a preferable embodiment the cold rolled strip contains at least 0.25% C and at least 0.03% Al. A lower limit of 0.25wt% is placed on C because below this level the desired combinations of strength and ductility may not be achieved.

In an embodiment the use of Si is preferred to that of Al such that a minimum silicon content of 1wt% and a max maximum aluminium content of 0.5 wt% is defined. Si provides substantial strengthening allowing the achievement of ultra high strength, more effectively suppresses carbide formation enabling longer isothermal holds without formation of large volumes of coarse iron carbides, and because it does not accelerate bainite formation to the same extent as Al thus preventing excessive formation of bainite and enabling higher strengths to be achieved.

Strength-Ductility data for a range of production C-Mn steels including ferritic forming steels and quenched martensitic steels have been used to generate a base-line strength-ductility decay for conventional strip steels. The data conform to the expression: ${e}_{calculated} = k ⁢ \frac{1}{\sqrt{{UTS}^{3}}}$
where e_{calculated} is the total elongation (expressed as % engineering strain), UTS is the ultimate tensile strength and k is a constant which for tensile test pieces with 80 mm gauge and thickness 1 mm is 250000.

If elongations are measured at different gauge or thickness then they must be converted to an equivalent elongation at 80mm gauge and 1mm thick or the above expression must be fit to base-line data measured at that alternative gauge/thickness combination using appropriate values of the constants. Conversion of tensile ductility can be performed using accepted procedures (ISO Norm 2566/1-2) when the geometries corresponding to the measured and to be calculated elongations are know: ${e}_{2} = {e}_{1} {\left(\frac{{L}_{1}}{{L}_{2}}\cdot \frac{\sqrt{{A}_{2}}}{\sqrt{{A}_{1}}}\right)}^{m}$
Where e2 is the required elongation for a gauge length of L₂ with a cross section of A₂, e₁ is the known elongation measured for a gauge length of L₁ with a cross section of A₁ and the exponent m is a material constant here assumed to be equal to 0.4.

In an embodiment the quenched and partitioned steel has an e-ratio of at least 1.8 wherein the e-ratio is defined as e_{measured}/e_{calculated} and wherein e_{mulated} is calculated according to equation (1) and wherein e_{measured} is the elongation measured from an 80mm gauge length sample at 1mm thick (or measured at some other geometry and converted to an equivalent elongation on an 80mm gauge at 1mm thick using expression (2)).

In an embodiment the tensile strength of the steel according to the invention is at least 900 MPa. This strength regime is of interest since it provides significant opportunity for down-gauging and is a strength regime for which formability is most limited. Ductility levels are at least 1.8x or more than that of conventional C-Mn steels at equivalent strength.

Preferably the yield to tensile strength ratio is 0.6 or higher. More preferably the ratio is at least 0.65 or even higher. Low yield to tensile strength ratios are associated with poor bendability and edge cracking sensitivity. Performance is often dependent on yield strength, anti-intrusion components for instance require high yield strength. High yield to tensile strength ratios ensure strength uniformity in the formed part, especially in forming operations which apply localised strain such as bending, or hole expansion.

In a preferred embodiment of the invention the metal or metal alloy coating is zinc, aluminium, magnesium or alloys thereof. Hereby the steel is afforded sacrificial corrosion protection since the zinc and aluminium will oxidise in preference to iron in the steel.

It was stated above that it is preferred that the partitioning temperature and time are chosen such as to optimise the enrichment of carbon in the austenite but without creation of deleterious microstructures during the isothermal hold. The temperature and time can be determined using dilatometry as follows:
First, fully austenitise a sample and apply a fast cool to room temperature to determine the fraction of martensite as a function of temperature below Ms. This allows to select an appropriate fraction of martensite as a function of the quench temperature. For this selected quench temperature the range of time-temperature partitioning combinations that deliver the correct stabilisation of austenite can be determined as follows. Cool a fully austenitized specimen to the selected quench temperature T₂ to produce the desired fraction of austenite and martensite and subsequently reheat the sample to a selected partitioning temperature T₃ and hold the sample at this temperature for a certain partitioning time t₂. The value of t₂ may be between 10 and 500 seconds, but for practical purposes in commercial annealing lines t₂ is preferably in the range of 20 to 180 s or even 20 to 100 s. After the partitioning step the specimen can be cooled naturally or acceleratedly to room temperature; no fast quench is needed. If during this cooling the dilatation curve shows that the martensite formation re-starts at a temperature in the range from (Ms - 20) to 120°C, then a correct degree of stabilisation has been achieved. In the case that the martensite formation recommences at a temperature <120°C, it means that the stabilisation is too strong and the martensite has a very high carbon content compared to the bulk concentration. In the other case that the martensite formation recommences at a temperature less than 20°C below Ms the stabilisation is not sufficient. This experiments needs to be repeated for different partitioning times to find the times corresponding the two limiting boundary conditions for the chosen partitioning temperature.

By varying the partitioning temperature T₃ and repeat above the required partitioning time will also vary. Increasing the partitioning temperature results in a decrease in partitioning time t₂ and to a higher degree of tempering of the martensite formed during the quench.

In a preferred embodiment of the invention the metallic coating is provided by hot-dip galvanising or by electro-galvanising.

### BRIEF DESCRIPTION OF THE DRAWINGS ,

The invention will now be elucidated by way of example making reference to the accompanying figures and examples.

Figure 1 shows the schematic annealing schedule indicating the meaning of T₁, T₂ and T₃, t₁ and t₂, and of CR1 and CR2.

Figure 2a and 2b show a set of result of the dilatometric experiments to determine the quench temperature and the partitioning time. Figure 2a shows the temperature as a function of time for a steel having 3.5% Mn which was quenched to a quench temperature of 280°C and reheated to a partitioning temperature of 330°C (triangle) and 440°C (circle). The sample was held at the partitioning temperature for 20 seconds. The quenching temperature resulting in the required amount of martensite is determined on the basis of the base curve (NC-III, square). Figure 2b shows the dilatation of the samples for these conditions. The base curve, with a full quench to room temperature allows to determine Ms (about 315°C). The partitioning step for 20s at 330°C shows no dilation of the sample, which means that no bainite is formed, carbon is partitioned and the martensite is only marginally tempered. The transformation to martensite re-starts at temperatures lower than the quench temperature of 280°C, namely at 250°C, which indicates that the austenite has been stabilized due to carbon partitioning. Increased partition times at 330°C show that the transformation to martensite re-starts at lower temperatures than 250°C. The dilation observed during annealing of the sample for 20s at 440°C means that bainite is formed. Concurrently, carbon is partitioned and the martensite is tempered. The consequence of this high partitioning temperature is that the martensite is severely tempered. Due to the bainitic transformation and the carbon partitioning the austenite is strongly enriched in carbon, which is reflected in the relatively low start temperature of the martensite of approximately 150°C during the second quench after the partitioning at 440°C. The latter martensite is very hard and brittle and therefore undesirable. By varying the partitioning time and the partitioning temperature the optimum combination can be determined.

Table 2 shows the results of various thermal cycles with the steels of Table 1. These results show that (I-VI):
I. The desired property balance is not achieved for processing with C and Mn additions at the level of current commercial TRIP Steels (composition G). G delivers a very large extension of ductility (typically 2.2 times that of a conventional C-Mn steel) at strengths ranging from 850 to 1050MPa. However, this is only true when the annealing temperature T₁ is chosen below the preferred range, (Ac₃-40 to Ac₃+40 such that a high fraction of ferrite is retained in the final structure. From table 2 it is apparent that, in these cases (cycles 31-32, although ductility is at the desired level, the ratio of YS to UTS drops below the desired level to approximately 0.4.
   When annealing is performed with T₁ within the claimed range, both direct quenching to room temperature and direct quenching to room temperature followed by an isothermal hold at a higher temperature (i.e. conventional quenching and tempering as in cycle 25) deliver strengths in the desired range but do not deliver ductility above the desired minimum level.
   When annealing is performed with T₁ within the claimed range (cycles 26-30 and 33) strengths in the range 1000-1300 MPa may be achieved but the desired level of ductility is not achieved.
   Processing variants annealed at T₁ within the claimed range, subsequently quenched to a low T₂ to give high fractions of martensite (in examples 85-93%) after the quench and followed by an isotherm at some higher temperature (table 3 cycles 28-30) to not deliver the desired level of ductility.
   Processing variants annealed at T₁ within the claimed range, subsequently quenched to a low T₂ to give high fractions of martensite after the quench followed by an isotherm at the same temperature (cycle 26) do not deliver the desired level of ductility.
   Processing variants annealed at T₁ within the claimed range, subsequently quenched to a high T₂ to give low fractions of martensite (in example 50%) after the quench followed by an isotherm at the same temperature (cycle 27) to not deliver the desired level of ductility.
II. Complete replacement of Si with Al delivers strength and ductility below the desired minima: Composition A when directly quenched to room temperature delivers strength in the desired range but ductility below the desired minimum (cycle 4). Composition A when quenched to a T₂ above the Mₛ temperature and subjected to isothermal holding at the same temperature delivers strength greatly below the desired range and ductility below the desired minimum (cycle 3). Composition A when quenched to a T₂ below the Mₛ temperature and subjected to isothermal holding at some higher temperature delivers strengths in the approximate range 950 to 1000MPa and ductilities below the desired minimum (thermal cycles 1-2).
III. Addition of C and/or Mn to levels beyond that found in current commercial trip steels does not enable the desired strength ductility balance to be achieved with conventional quench and temper process. For compositions B, C, D, E , F, and H utilising a direct quench or a direct quench followed by isothermal holding at some higher temperature (i.e. conventional quench and temper) delivers strengths in the desired range but ductility lower than the required minimum (cycles 9, 14, 25, 19, 24, 38).
IV. Addition of C and/or Mn enables the desired strength ductility balance to be achieved when T₂ is above the preferred range but only when the duration of the isothermal hold is unacceptably long for conventional process. Compositions B, C, D, F and H each enable the desired property range to be achieved even if T₂ is set such that no martensite is formed during the initial quench (cycles 8, 12, 13, 16, 17, 36 and 37) but in all cases the isothermal holding time at T₃ is unacceptably long to be practical or economical in a continuous annealing process.
V. Addition of C and/or Mn enables the desired strength ductility balance to be achieved when processing is carried out in the preferred manner using a quench temperature (T₂) below Ms and a suitable combination of isothermal holding temperature (T₃) and time. Compositions B, D and F each enable the desired property range to be achieved if T₂ is set such that the desired fraction of martensite is formed during the initial quench (cycles 6, 15, 22) and if an isothermal holding temperature (T₃) and the holding time at this temperature are set at suitable levels.
VI. C addition of higher than 0.4wt% leads to embrittlement when processing is carried out according to the preferred route. Compositions C and H each return effectively zero ductility results when subjected to processing involving a deep quench (low T₂) and isothermal hold times at T₃ sufficiently short for conventional CA process (cycles 10-11 and 34-35) due to the formation of brittle, high carbon martensite in the final structure.

## Claims

1. A method for producing a quenched and partitioned steel by providing a cold rolled and annealed steel strip containing (in weight %):
• 0.18 - 0.4% C
• 1.5 - 4.0% Mn
• 0.5 - 2.0% Si
• 0-1.5% Al
• 0-0.5% Mo
• 0-0.5% Ti
• 0 - 0.1% V
• 0 - 0.010% Nb
• 0 - 0.005% B
• 0 - 0.015% N
• 0 - 0.08% P
• 0 - 0.01% S
• 0-0.06% Sb
• 0-0.05% Ca
• 0 - 0.5%Cr
• 0-1.0% Ni
• the remainder being iron and unavoidable impurities.
wherein the annealing process comprises the following steps:
(i) reheating the cold rolled strip to an annealing temperature T₁ of between Ac₃-40 and Ac₃+80;
(ii) holding the strip at T₁ for an annealing time t₁ of between 10 and 200 seconds;
(iii) cooling the annealed strip at the critical cooling rate CR1 for avoidance of ferrite and pearlite formation to a quench temperature T₂ for producing a microstructure in the strip comprising a martensite fraction and a retained austenite fraction;
(iv) repartitioning annealing the cooled strip at a temperature T₃ for enriching the austenite in carbon by repartitioning the carbon from the martensite to the austenite fraction for a repartitioning time t₂ of between 20 and 500 seconds wherein the martensite fraction is between 60 and 90% of the microstructure at the start of the repartitioning annealing wherein (Ms-70) < T₃ ≤ (Ms+50)
(v) cooling the strip at a cooling rate CR2 to ambient temperature.

2. A method according to claim 1 wherein CR1 is at least 30°C/s.

3. A method according to claim 1 or 2 wherein the martensite fraction is at most 85% of the microstructure at the start of the repartitioning annealing.

4. A method according to any one of the preceding claims wherein
(Ac₃-40) < T₁ ≤ (Ac₃+50) for carbon between 0.18 - 0.3% C or
(Ac₃-20) < T₁ ≤ (Ac₃+30) for carbon between 0.3 to 0.4% C

5. A method according to any one of the preceding claims wherein T1 is above Ac3.

6. A method according to any one of the preceding claims wherein the cold rolled strip contains at most 0.5% Al.

7. A method according to any one of the preceding claims wherein the cold rolled strip contains at least 0.25% C and at least 0.01% Al.

8. A method according to any one of the preceding claims wherein T₂ equals T₃.

9. A method according to any one of claims 1 to 7 wherein T₂ is lower than T₃.

10. A method according to any one of the preceding claims wherein the cold-rolled and annealed strip is coated with one or more metallic layer(s), preferably wherein the step of providing the metallic coating is by hot-dip galvanising or electro-galvanising.

11. Steel strip produced by any one of the claims 1 to 10 wherein the steel has a microstructure containing at least 5% austenite, wherein the microstructure contains 60 to 90 % (in volume) of thermally treated martensite and wherein an e-ratio of at least 1.8 and a tensile strength (UTS) of at least 900 MPa, wherein the e-ratio is defined as e_{measured}/e_{calculated} and wherein e_{calculated} is calculated according to: ${e}_{calculated} = k ⁢ \frac{1}{\sqrt{{UTS}^{3}}}$ and wherein measured is the elongation measured from an 80mm gauge length sample at 1mm thick, or wherein e_{measured} is the elongation measured at some other geometry and converted to an equivalent elongation on an 80mm gauge at 1mm thick using: ${e}_{2} = {e}_{1} {\left(\frac{{L}_{1}}{{L}_{2}}\cdot \frac{\sqrt{{A}_{2}}}{\sqrt{{A}_{1}}}\right)}^{m}$

12. Steel strip according to claim 11 wherein the microstructure further contains one or more of bainite, martensite, tempered martensite, ferrite, fine carbides.

13. Steel strip according to claim 11 or 12 wherein the microstructure does not contain ferrite and/or coarse cementite.

14. Steel strip according to any one of claims 11 to 13 wherein the yield strength to tensile strength ratio is at least 0.6.

## Patentansprüche

1. Verfahren zum Herstellen von abgeschrecktem und partitioniertem Stahl durch Bereitstellen eines kaltgewalzten und geglühten Stahlbandes, der (in Gew.-%) folgendes enthält:
• 0,18 - 0,4 % C
• 1,5 - 4,0 % Mn
• 0,5 - 2,0 % Si
• 0 - 1,5% Al
• 0 - 0,5% Mo
• 0 - 0,5% Ti
• 0-0,1%V
• 0 - 0,010 % Nb
• 0 - 0,005 % B
• 0 - 0,015 % N
• 0 - 0,08 % P
• 0-0,01 %S
• 0 - 0,06 % Sb
• 0 - 0,05 % Ca
• 0-0,5%Cr
• 0 - 1,0 % Ni
• wobei der Rest Eisen und unvermeidbare Verunreinigungen ist,
wobei der Glühprozess die folgenden Schritte umfasst:
(i) Wiedererhitzen des kaltgewalzten Bandes auf eine Glühtemperatur T₁ zwischen Ac₃ - 40 und Ac₃ +80;
(ii) Halten des Bandes auf T₁ über eine Glühzeit t₁ zwischen 10 und 200 Sekunden;
(iii) Kühlen des geglühten Streifens mit der kritischen Kühlrate CR1, um eine Bildung von Ferrit und Perlit zu vermeiden, auf eine Abschreckungstemperatur T₂, um eine Mikrostruktur in dem Band zu erzeugen, die einen Martensitanteil und einen Restaustenitanteil umfasst;
(iv) repartitionierendes Glühen des gekühlten Bandes auf einer Temperatur T₃, um das Austenit in Kohlenstoff anzureichern durch Repartitionierung des Kohlenstoffs aus dem Martensit auf den Austenitanteil über eine Repartitionierungszeit t₂ zwischen 20 und 500 Sekunden, wobei der Martensitanteil zu Beginn des repartitionierenden Glühens zwischen 60 und 90 % der Mikrostruktur liegt, wobei (Ms-70) < T₃ ≤ (Ms+50);
(v) Kühlen des Bandes mit einer Kühlrate CR2 auf Umgebungstemperatur.

2. Verfahren nach Anspruch 1, wobei CR1 mindestens 30 °C/s beträgt.

3. Verfahren nach Anspruch 1 oder 2, wobei der Martensitanteil zu Beginn des repartitionierenden Glühens höchstens 85% der Mikrostruktur beträgt.

4. Verfahren nach einem der vorstehenden Ansprüche, wobei: $\left({AC}_{3}-40\right) < {T}_{1} \leq \left({AC}_{3}+50\right) für Kohlenstoff zwischen 0 , 18 - 0 , 3 % C ;$
oder $\left({AC}_{3}-20\right) < {T}_{1} \leq \left({AC}_{3}+30\right) für Kohlenstoff zwischen 0 , 3 bis 0 , 4 % C .$

5. Verfahren nach einem der vorstehenden Ansprüche, wobei T₁ größer ist als Ac₃.

6. Verfahren nach einem der vorstehenden Ansprüche, wobei der kaltgewalzte Band höchstens 0,5 % Al enthält.

7. Verfahren nach einem der vorstehenden Ansprüche, wobei der kaltgewalzte Band mindestens 0,25 % C und mindestens 0,01 % Al enthält.

8. Verfahren nach einem der vorstehenden Ansprüche, wobei T₂ gleich T₃ ist.

9. Verfahren nach einem der Ansprüche 1 bis 7, wobei T₂ kleiner ist als T₃.

10. Verfahren nach einem der vorstehenden Ansprüche, wobei der kaltgewalzte und geglühte Band mit einer oder mehreren metallischen Schicht(en) überzogen ist, wobei der Schritt des Bereitstellens des metallischen Überzugs vorzugsweise durch Feuerverzinkung oder galvanische Verzinkung erfolgt.

11. Stahlband, der durch ein Verfahren nach einem der Ansprüche 1 bis 10 erzeugt worden ist, wobei der Stahl eine Mikrostruktur aufweist, die mindestens 5 % Austenit enthält, wobei die Mikrostruktur 60 bis 90 % (Volumenprozent) wärmebehandeltes Martensit enthält, und wobei ein e-Verhältnis von mindestens 1,8 und eine Zugfestigkeit (UTS) von mindestens 900 MPa gegeben sind, wobei das e-Verhältnis definiert ist als e_{gemessen}/e_{berechnet}, und wobei e_{berechnet} wie folgt berechnet wird: ${e}_{berechnet} = k ⁢ \frac{1}{\sqrt{{UTS}^{2}}}$ und wobei e_{gemessen} der an einem Probenstück mit einer Dicke von 1 mm gemessenen Elongation bei einer Messlänge von 80 mm entspricht, oder wobei e_{gemessen} der an einer anderen Geometrie gemessenen Elongation entspricht, und umgewandelt in eine äquivalente Elongation bei einer Messlänge von 80 mm und einer Dicke von 1 mm unter Verwendung von: ${e}_{2} = {e}_{1} {\left(\frac{{L}_{1}}{{L}_{2}}⋅\frac{\sqrt{{A}_{2}}}{\sqrt{{A}_{1}}}\right)}^{m}$

12. Stahlband nach Anspruch 11, wobei die Mikrostruktur ferne eines oder mehrere der aus Bainit, Martensit, angelassenem Martensit, Ferrit, feinen Carbiden enthält.

13. Stahlband nach Anspruch 11 oder 12, wobei die Mikrostruktur kein Ferrit und/oder grobes Cementit enthält.

14. Stahlband nach einem der Ansprüche 11 bis 13, wobei das Verhältnis der Streckgrenze zur Zugfestigkeit mindestens 0,6 beträgt.

## Revendications

1. Procédé de production d'un acier trempé et partitionné en utilisant une bande d'acier laminée à froid et recuite contenant (en % en poids) :
• 0,18 - 0,4 % C
• 1,5 - 4,0 % Mn
• 0,5 - 2,0 % Si
• 0 - 1,5 % Al
• 0 - 0,5 % Mo
• 0 - 0,5% Ti
• 0 - 0,1 % V
• 0 - 0,010 % Nb
• 0 - 0,005 % B
• 0 - 0,015 % N
• 0 - 0,08 % P
• 0-0,01 %S
• 0 - 0,06 % Sb
• 0 - 0,05 % Ca
• 0 - 0,5 % Cr
• 0-1,0% Ni
• le reste étant du fer et des impuretés inévitables
dans lequel le procédé de recuit comprend les étapes suivantes :
(i) réchauffer la bande laminée à froid à une température de recuit T₁ comprise entre Ac₃-40 et Ac₃+80 ;
(ii) maintenir la bande à T₁ pendant un temps de recuit t₁ compris entre 10 et 200 secondes ;
(iii) refroidir la bande recuite à la vitesse de refroidissement critique CR1 pour éviter la formation de ferrite et de perlite à une température de trempe T₂ pour produire une microstructure dans la bande comprenant une fraction de martensite et une fraction d'austénite résiduelle ;
(iv) recuire pour repartitionnement la bande refroidie à une température T₃ pour enrichir l'austénite en carbone en repartitionnant le carbone à partir de la martensite à la fraction d'austénite pendant un temps de repartitionnement t₂ compris entre 20 et 500 secondes, dans lequel la fraction de martensite est comprise entre 60 et 90 % de la microstructure au début du recuit de repartitionnement dans lequel (Ms-70) < T₃ ≤ (Ms+50) ;
(v) refroidir la bande à une vitesse de refroidissement CR2 à température ambiante.

2. Procédé selon la revendication 1, dans lequel CR1 est d'au moins 30 °C/s.

3. Procédé selon la revendication 1 ou 2, dans lequel la fraction de martensite est au maximum de 85 % de la microstructure au début du recuit de partitionnement.

4. Procédé selon l'une quelconque des revendications précédentes, dans lequel : $\left({AC}_{3}-40\right) < {T}_{1} \leq \left({AC}_{3}+50\right) pour le carbone entre 0 , 18 - 0 , 3 % C$
ou $\left({AC}_{3}-20\right) < {T}_{1} \leq \left({AC}_{3}+30\right) pour le carbone entre 0 , 3 à 0 , 4 % C$

5. Procédé selon l'une quelconque des revendications précédentes, dans lequel T₁ est supérieure à Ac3.

6. Procédé selon l'une quelconque des revendications précédentes, dans lequel la bande laminée à froid contient au maximum 0,5 % d'Al.

7. Procédé selon l'une quelconque des revendications précédentes, dans lequel la bande laminée à froid contient au moins 0,25 % de C et au moins 0,01 % d'Al.

8. Procédé selon l'une quelconque des revendications précédentes, dans lequel T₂ est égale à T₃.

9. Procédé selon l'une quelconque des revendications 1 à 7 dans lequel T₂ est inférieure à T₃.

10. Procédé selon l'une quelconque des revendications précédentes, dans lequel la bande laminée à froid et recuite est revêtue d'une ou plusieurs couche(s) métallique(s), de préférence dans lequel l'étape de fourniture de revêtement métallique est par galvanisation à chaud ou électro-galvanisation.

11. Bande d'acier produite par l'une quelconque des revendications 1 à 10, dans laquelle l'acier a une microstructure contenant au moins 5 % d'austénite, dans laquelle la microstructure contient de 60 à 90 % (en volume) de martensite traitée thermiquement et dans laquelle un e-rapport est d'au moins 1,8 et une résistance à la traction (UTS) d'au moins 900 MPa, dans laquelle l'e-rapport est défini comme e_{measured}/e_{calculated} et dans laquelle e_{calculated} est calculé selon : ${e}_{calculated} = k ⁢ \frac{1}{\sqrt{{UTS}^{3}}}$
et dans laquelle e_{measured} est l'allongement mesuré à partir d'un échantillon de longueur de calibre de 80 mm à 1 mm d'épaisseur, ou dans laquelle e_{measured} est l'allongement mesuré à une autre géométrie et converti en un allongement équivalent sur un calibre de 80 mm à 1 mm d'épaisseur à l'aide de : ${e}_{2} = {e}_{1} {\left(\frac{{L}_{1}}{{L}_{2}}\cdot \frac{\sqrt{{A}_{2}}}{\sqrt{{A}_{1}}}\right)}^{m}$

12. Bande d'acier selon la revendication 11, dans laquelle la microstructure contient en outre un ou plusieurs parmi la bainite, la martensite, la martensite trempée, la ferrite, les carbures fins.

13. Bande d'acier selon la revendication 11 ou 12, dans laquelle la microstructure ne contient pas de ferrite et/ou de cémentite grossière.

14. Bande d'acier selon l'une quelconque des revendications 11 à 13, dans laquelle le rapport limite d'élasticité/résistance à la traction est d'au moins 0,6.
